

1

2,845,349

## PHOTOGRAPHIC DEVELOPERS

George Schwarz, Glen Head, N. Y., assignor to Powers Chemco, Inc., Glen Cove, N. Y., a corporation of New York

No Drawing. Application September 7, 1955  
Serial No. 533,010

3 Claims. (Cl. 96—66)

The present invention relates to novel and improved photographic developers.

Objects and advantages of the invention will be set forth in part hereinafter and in part will be obvious herefrom, or may be learned by practice with the invention, the same being realized and attained by means of the steps, process and compositions and improvements herein shown and described.

Photographic developers, especially those having a relatively low concentration of sulfite ions have very poor keeping qualities and are subject to rapid oxidation when exposed to the atmosphere. Under certain unfavorable conditions even high sulfite concentrations in developers do not prevent rapid aerial oxidation, for example when the water contained in the developer is contaminated with very small amounts of iron, copper, or other heavy-metal containing ionic compounds, and in normal practice it is difficult and seldom feasible to provide for water free of such heavy-metal ionic compounds.

Developers are also subject to other types of deterioration, particularly in deep tanks, such as are used for the commercial processing of roll film. Often such developers are subjected to deterioration by micro-organisms which reduce the sulfite to sulfide and cause putrefaction of the developer and fogging of the film. Most photographic developers also react with the impurities in the water to form precipitates of calcium and magnesium salts and cause the formation of cloudy solutions, which can be avoided only by the use of specially purified water which is not generally available for the purpose.

The present invention has for its object the provision of a photographic developer which has superior keeping qualities, is not readily susceptible to aerial oxidation, and which does not suffer from the use of the ordinary water which is generally available for the preparation of such a developer. A further object of the invention is the provision of a developer which is not readily susceptible to putrefaction and which, in use, reduces the fogging which often occurs in the commercial use of conventional developers. Still another object is the provision of a developer which does not seriously suffer from being made up with relatively hard water, or water containing normal amounts of copper, iron or other heavy-metal ionic compounds.

The various disadvantages of the conventional developers, as set forth above, can be greatly reduced and largely avoided by the addition to the conventional photographic developer of relatively small amounts of an organic cyclic compound which is water-soluble and contains the atomic grouping



in a quantity of from about 0.01 to about 0.25 mol per litre of developer, preferably about 0.1 mol per litre, although the amount of such cyclic compound may be varied widely within the limits given. Preferably, the water soluble salts of kojic acid or the acid itself is used, in quantities of from about 2 grams to as much as 30 or 35 grams per litre, the pH of the developer being ad-

2

justed as desired in view of the quantity of kojic acid or kojic acid salt used, so that the alkalinity (or acidity) of the developer is substantially the same as would be used with a conventional developer.

5 The kojic acid and its related compounds are to be distinguished from the compounds related to ascorbic acid which do not contain the  $\gamma$ -pyrone grouping, although they do contain the

10



group. Such compounds are much less effective and more expensive than those which contain both the  $\gamma$ -pyrone group and the above-mentioned functional group, such as kojic acid.

15 It will be understood that the foregoing general description and the following detailed description as well are exemplary and explanatory of the invention but are not restrictive thereof.

20 The following are specific examples of various preferred photographic developers in accordance with the present invention and which illustrate the principles of the invention.

### Example 1.—Metol-hydroquinone developer

25

|                                     | Grams |
|-------------------------------------|-------|
| N-monomethylparaminophenol sulphate | 7     |
| Hydroquinone                        | 7     |
| Sodium sulfite, anhydrous           | 50    |
| Sodium carbonate, anhydrous         | 35    |
| 30 Potassium bromide                | 1     |
| Water, q. s. ad. 1 litre.           | 1     |
| Kojic acid                          | 2     |

35 If the water is relatively hard, the kojic acid is preferably dissolved in the water before the remainder of the developer is dissolved in the water, thereby avoiding the formation of a calcium or magnesium precipitate. Whether or not the kojic acid is first dissolved in the water, the developer is protected against reduction of the sulfite to sulfide by micro-organisms which contaminate the water.

### Example 2.—Tanning developer

40 A tanning developer with a low sulfite concentration, which can be omitted for certain purposes, if desired, has its tray life doubled or tripled with respect to a similar developer which does not include the addition of the kojic acid. Such a developer comprises:

|                              | Grams |
|------------------------------|-------|
| Catechol                     | 5     |
| 50 Sodium sulfite (optional) | 3     |
| Potassium carbonate          | 30    |
| Kojic acid                   | 10    |
| Water, q. s. ad. 1 litre.    | 1     |

55 The sodium sulfite may be omitted, decreased or increased, if desired, and the catechol may be partially or completely replaced by pyrogallol or hydroquinone. The kojic acid may be varied from 2 grams to as much as 30 or 55 grams, although when higher amounts of kojic acid are used, it may be desirable to increase slightly the amount of alkali so as to maintain the pH within the desired limits.

### Example 3.—Alkali-free (amidol) developer

60 An alkali free developer can be made with amidol which has a tray life approximately double that of a similar developer not including the kojic acid.

|                              | Grams |
|------------------------------|-------|
| Amidol                       | 5     |
| 65 Sodium sulfite            | 50    |
| Kojic acid                   | 15    |
| 70 Water, q. s. ad. 1 litre. | 1     |

*Example 4.—Extreme contrast (lithographic) developer*

|                               | Grams |
|-------------------------------|-------|
| Sodium formaldehyde-bisulfite | 40    |
| Hydroquinone                  | 25    |
| Kojic acid                    | 10    |
| Sodium carbonate              | 38    |
| Potassium bromide             | 2     |
| Water, q. s. ad. 1 litre.     |       |

Such a developer has a greatly improved tray life over a similar developer prepared without kojic acid, as well as with respect to a similar developer in which the pH was made equivalent by the addition of boric acid in place of the kojic acid. The kojic acid not only serves to maintain the strength of the developer over a longer period of time, but also minimizes the discoloration of the developer. The kojic acid concentration is not critical and may be varied from 1 gram to 25 grams per litre if the acidity is properly adjusted by using more or less of the sodium carbonate, or otherwise.

*Example 5.—Color-coupling developer*

A color-coupling developer with increased resistance against aerial oxidation and color fog may be prepared as follows:

|                                        | Grams |
|----------------------------------------|-------|
| Paradimethylaminoaniline hydrochloride | 10    |
| Sodium sulfite                         | 5     |
| Sodium carbonate                       | 35    |
| Kojic acid                             | 10    |
| α-Naphthol                             | 5     |

While the developers of the present invention are preferably packaged for sale in the dry form, they may be packaged as a concentrate, in well sealed bottles and preferably prepared with a small amount of distilled water, ready for dilution to the desired concentration. When packaged dry, the chemicals are preferably separated into two groups, one group comprising the developing agents, the kojic acid or equivalent thereof and the sulfite, while the other group comprises the remainder of

the chemicals, such as the alkaline salt, e. g. sodium carbonate. It is of little importance in which group the potassium bromide is included, but it is always advantageous to have the developing agent in the same package with the sulfite.

Thus, the developer of Example 1 would preferably be packaged dry as a first package comprising the mono-methylparaminophenol sulfate, sodium sulfite and kojic acid, while the second package would comprise the sodium carbonate, hydroquinone and potassium bromide. Likewise, the developer of Example 2 would preferably have the second package include only the potassium carbonate, with the remainder of the ingredients in the first package.

The quantity of water given in all of the above formulae is the preferable quantity, and of course, it may be widely varied in accordance with standard photographic techniques, depending upon the effect desired from the developer.

The invention in its broader aspects is not limited to the specific steps, process and compositions shown and described but departures may be made therefrom within the scope of the accompanying claims without departing from the principles of the invention and without sacrificing its chief advantages.

What is claimed is:

1. A photographic developer comprising an organic silver-halide developing agent, an alkali sulfite and an amount sufficient to form from 1 to 35 grams per liter when dissolved in water of a compound selected from the group consisting of kojic acid and its water soluble salts.
2. A photographic developer as claimed in claim 1 in which the alkali is sodium formaldehyde bisulfite and the developing agent is hydroquinone.
3. A photographic developer as claimed in claim 2 in which the compound is kojic acid.

**References Cited in the file of this patent**

40 Pontius: PSA Journal, Section B, September 1951, pp. 76-79.